

## UNITED STATES PATENT OFFICE

2,202,092

## PROCESS OF FINISHING LEATHER

Leon B. Conant, Boston, Mass.

No Drawing. Application April 4, 1939,  
Serial No. 265,973

4 Claims. (Cl. 149—6)

This invention relates to an improvement in the heat treatment of leather having application, in particular, to its preparation and character immediately preceding its impregnation or permeation by liquid oleaginous material. The primary purpose of this invention is to give effect to the saturation of the leather fibre by a hot oleaginous liquid filler by removing, prior to its immersion therewith, all of the hygroscopic moisture in the leather by an adequate dehydration and pre-heating thereof.

The tanner and currier of leather, is afraid of the effect of heat, or rather of its energy, upon leather with the result that leather, heretofore, has never been freed of its hygroscopic water content prior to its stuffing with fillers. Hence the leather fibres have not had direct contact with the impregnating finishing oils; instead the liquid wax, or the oils, as ordinarily introduced, merely clog the pores and interstices of the leather. That is to say, the tanned fibres of the leather during its currying and stuffing, although dried out moderately on occasion, are never dried enough to complete their dehydration and pre-heating to adaptation for saturation by oils, whether applied hot or cold. For example, 200° F. is an extreme rarely used in drying leather in a tannery; 212° F. has been considered prohibitive. Yet, neither one can effect sufficient dehydration for any permanent impregnation by oil. It is my purpose to employ heat as high as 300° F. or, more or less as required, to make the leather absolutely anhydrous and hot in complete adaptation for its impregnation, preferably by heated oleaginous liquid filler applied thereto while at approximately equal temperature with the leather itself.

In my U. S. Patents Numbered 1,719,101, 1,769,943, 1,787,145, 1,934,038, and 2,032,471, each entitled Process of vulcanizing rubber to leather, I have described the dehydration and pre-heating of leather to adaptation for its union with rubber composition during hot vulcanization whereby its original character and quality are in no way injured or impaired. Under modern methods most rubber compositions are vulcanized at 260° F. and up. 300° F. is a fair average. By the use of the patented processes aforesaid, leather is adaptable to these and to even higher vulcanizing temperatures. Hence, my experience of many years in pre-heating leather to adaptation for the dry heat of hot vulcanization at elevated temperatures enabled me to discover and perfect this process of pre-heating leather to complete preparation and adaptation for im-

pregnation by molten paraffin wax or other oleaginous liquids. But, whereas, the application of the dry heat of vulcanization permits that the pre-heated body temperature of the leather be substantially less than its own, the pre-heated leather to be adapted for immersion in a hot oleaginous bath should possess approximately at least an equivalent temperature to that of the bath when placed therein. Preferably, the heated leather is hotter than the bath, and so really cools off moderately therewith. The elevated body temperature of the leather as described assures rapid and beneficial absorption of the hot oleaginous liquid. Therefore, this new process effects real saturation of the leather fibres and thereby prevents the leather from cracking during wear. Ordinarily leather uppers crack because the oleaginous fillers are put in on top of the hygroscopic water already present therein. Such practice of finishing upper leather for instance, only places the oils between the moisture laden fibres. Actually, the semi-moist fibres are not truly impregnated. Water and oil do not mix. Consequently, when shoes are cleaned the oleaginous filler in the uppers is washed out of the leather pores until finally none is left therein and the uppers crack. Accordingly this process is designed primarily to eliminate the hygroscopic water present in leather by heating the same to complete dehydration, and then while so heated, introducing its quota of oleaginous content therewith in intimate association with the fibres thereof. It should be understood, however, that my preference is to impregnate the leather with hot paraffin wax blended with rubber under heat and eventually coagulated as incorporated therein.

The basic principle of my process requires that the leather must be pre-heated to complete dehydration so that its fibres shall be absolutely free of all hygroscopic moisture when immersed in the oleaginous bath. Moreover, whatever the temperature of the bath may be, I prefer the leather be hotter. Also, I prefer that the bath be heated well above 220° F. because the hotter the elevated temperature of the bath the quicker the impregnation of the hot leather is completed. In addition I propose, on occasion, to use compounded rubber composition in the hot oleaginous liquid and beside dispersing or dissolving it in the molten paraffin, to vulcanize it therewith in the presence of sulphur and other suitable agents. Also, I plan if needed to apply heat and pressure to the impregnated leather.

In making my process effective I take leather

of any description such as upper, sole, upholstery, etc., or a split thereof, as tanned, but preferably not stuffed with fillers, and pre-heat it to suit above 220° F. and while so heated immerse it or 5 otherwise impregnate it with an oleaginous liquid. If the bath comprises a blend of paraffin and rubber, it may be heated to approximate the body-heat of the leather and either crude or compounded rubber may be used. If a compound, 10 the same may be adapted to be vulcanized by the hot oleaginous liquid during its dispersion therein, by elevating the temperature thereof to suit, or, the hot oleaginous liquid may be kept at a sub-vulcanizing temperature while the 15 rubber compound is dissolved therein and while the leather is being impregnated and then upon removal from the bath, the saturated leather may have the rubber cured therein with heat and pressure. When now the leather has become impregnated to suit, it is removed from the paraffin-rubber bath and compressed under heat and pressure or simply allowed to dry out. When dry 20 an improved durable and serviceable leather is at hand. It is understood that any variety of compounding may be used in blending crude rubber or rubber composition with the molten paraffin or tallow or other fat, or a combination thereof, as desired. If colored leather is being treated care must be used not to destroy its finish. Such 25 leather should be dipped briefly. Incidentally, my pre-heating of leather to adaption helps to preserve its color. Oak tanned sole leather as heated in advance by my process may be readily treated in the hot oleaginous bath. Otherwise 30 it would be ruined. It too should be handled so as to retain its natural color. Chrome sole leather immersed in the bath is no problem.

The elevated temperatures employed by my process for both leather and the paraffin-rubber bath permit saturation ordinarily in less than one-half hour. In contrast, the prior art recites three to four hours as requisite. 5

It is understood that the application of this process comprises its use in the treatment of any fibrous material; for example, wood, paper, fabric, leather, etc.

This process may be summarized as comprising 10 the impregnation of hot dehydrated leather by heated oleaginous liquid.

I claim:

1. The process comprising pre-heating leather at a temperature above, 220° F. and removing all 15 of its hygroscopic water content and then, while so heated, impregnating it with hot oleaginous liquid.

2. The process comprising pre-heating leather at a temperature above 220° F. and eliminating 20 all of its hygroscopic water content and then, while so heated, immersing it for impregnation in a hot oleaginous liquid heated to a lower temperature.

3. The process comprising pre-heating leather 25 at a temperature above 220° F. and removing all of its hygroscopic water content, and then, while so heated, immersing it in a hot oleaginous bath comprising a blend of paraffin and rubber.

4. The process comprising pre-heating leather 30 at a temperature above 220° F. and removing all of its hygroscopic water content and then, while so heated, immersing it in a hot oleaginous bath of vulcanizable rubber composition and paraffin. 35

LEON B. CONANT.